# EUROPEAN PATENT SPECIFICATION

(11) **EP 1 080 266 B1**
(45) Date of publication and mention of the grant of the patent: **19.02.2003**
(21) Application number: 99924321.5
(22) Date of filing: 18.05.1999
(51) Int. Cl.: D21F 11/00

(54) **PROCESS FOR INCREASING BULK OF FORESHORTENED FIBROUS WEB**
VERFAHREN ZUR ERHÖHUNG DES VOLUMENS VON EINER GEKREPPTEN FASERSTOFFBAHN
PROCEDE D'AUGMENTATION DU VOLUME DE TOILE DE FIBREUSE RACCOURCIE

(30) Priority: 18.05.1998 US 80738; 18.05.1998 US 80863
(43) Date of publication of application: 07.03.2001
(73) Proprietor: THE PROCTER & GAMBLE COMPANY, Cincinnati, Ohio 45202 (US)
(72) Inventor: RICHARDS, Mark, R., Middletown, OH 45042 (US)
(74) Representative: Kohol, Sonia
(86) International application number: US9910973
(87) International publication number: WO99060206

(56) References cited:
- WO-A-93/11301
- GB-A- 1 220 070
- US-A- 5 702 571

## Description

### FIELD OF THE INVENTION

The present invention is related to processes and apparatuses for making strong, soft, absorbent fibrous webs. More particularly, the present invention is concerned with foreshortened fibrous webs.

### BACKGROUND OF THE INVENTION

Fibrous structures, such as paper webs, are produced by a variety of processes. For example, paper webs may be produced according to commonly-assigned U, S. Patents: 5,556,509, issued Sept. 17, 1996 to Trokhan et al.; 5,580,423, issued Dec. 3, 1996 to Ampulski et al.; 5,609,725, issued Mar 11, 1997 to Phan; 5,629,052, Issued May 13, 1997 to Trokhan et al.; 5,637,194, issued June 10, 1997 to Ampulski et al.; and 5,674,663, Issued Oct 7, 1997 to McFarland et al. Paper webs may also be made using through-air drying processes as described in commonly-assigned U.S. Patents 4,514,345, issued April 30, 1985 to Johnson et al.; 4,528,239, Issued July 9 to Trokhan, 1985; 4,529,480, issued July 16, 1985 to Trokhan; 4,637,859, issued January 20, 1987 to Trokhan; and 5,334,289, issued August 2, 1994 to Trokhan et al.

WO 93/11301 A, commonly assigned to The Procter & Gamble Company, discloses a cellulosic fibrous structure, particularly consumer products such as toilet tissue, facial tissue or a paper towel, having a plurality of protuberances extending outwardly from each face of the cellulosic fibrous structure. The protuberances may extend bilaterally outwardly from the plane of the cellulosic fibrous structure in both directions. The bilaterally extending protuberances increase the caliper and texture of the consumer product embodied in the cellulosic fibrous structure. The protuberances may be Induced by mechanical embossing or by fluid embossing. This application also discloses a fluid embossing process for making such cellulosic fibrous structures.

U.S. Patent No. 5,702,571 discloses tissue sheets, such as are useful for facial or bath tissue, which are embossed with a fine scale embossing pattern to Increase bulk with a minimal loss in strength. The fine scale embossing pattern contains at least about 15 discrete intermeshing embossing elements per square centimeter and can enable the tissue manufacturer to produce premium quality tissue having adequate softness, bulk and strength from conventional tissue basesheets without layering or throughdrying equipment.

GB 1,220,070 discloses a device for the continuous manufacture of patterned paper. The device comprises a movable machine-wire means, means for distributing liquid stock onto said machine-wire means at uniform thickness, first dewatering means for removing the bulk of the moisture in the liquid stock distributed on said wire means so as to form a continuous wet-web of uniform thickness, patterning belt means having perforations and movable at the same speed as said machine-wire means, means for ejecting water under pressure through said perforations onto said wet web, at water pressure equalising means disposed below said water-ejecting means and above the lower run of said patterning belt means, second dewatering means for removing ejected water after said ejected water has passed through the perforations, the wet-web and the machine wire means, and means for heating the wet-web to produce dry patterned paper. The patterned paper thus dried, may be subjected further to a mechanical cockling treatment to make the paper shrinkable by alkylamine. The patterned paper according to that Specification may also be laminated with non-patterned paper by superimposing the patterned paper on the wet-web and rolling them together under pressure.

Foreshortening of a fibrous webs may be used to increase the web's caliper, absorbency and softness. Foreshortening refers to reduction in length of a dry web, resulting from application of energy to the web. Typically, during foreshortening, rearrangement of the fibers in the web occurs, accompanied by at least partial disruption of fiber-to-fiber bonds. As a result of foreshortening, micro-folds, commonly called "crepe" are formed in the web.

It has been discovered that the increase In caliper, or bulk, of the foreshortened web may further be achieved by relaxing, at least partially, the crepe in the web. It has been further found that the crepe can be relaxed in pre-selected portions of the web such that the rest of the web, not affected by the crepe relaxation, retains the quality of the foreshortened web.

Accordingly, it is a subject of the present invention to provide a novel process for increasing bulk of the foreshortened web by relaxing the web's crepe in the selected portions of the web. It is another object of the present invention to provide an apparatus for Increasing bulk of the foreshortened web by relaxing the web's crepe In the selected portions of the web.

### SUMMARY OF THE INVENTION

The present invention provides a process and an apparatus for increasing caliper/bulk of a foreshortened fibrous web by causing selected micro-regions, or portions, of the foreshortened web to relax crepe therein, thereby expanding outwardly from the general plan of the web. The process comprises the steps of providing a foreshortened web comprising crepe and having a general plane; and adding moisture to the web or to at least the web's selected portions, thereby causing relaxation of the crepe in the selected portions and their expansion outwardly from the general plane of the web, while retaining the crepe in the rest of the web. The preferred apparatus comprises two mutually opposite surfaces designed to receive and restrain the foreshortened web therebetween, at least one of the surfaces having a plurality of fluid-permeable expansion conduits therethrough; a means for moistening the web or at least its selected portions corresponding to the expansion conduits when the foreshortened web is disposed between the two surfaces; and a means for creating a temperature differential between the two surfaces such that when the web is restrained between the surfaces, the temperature differential is sufficient to cause the moisture added to the web to move through the web in the direction from one surface toward the other, thereby relaxing crepe in the selected portions of the web and causing the selected portions to expand through the expansion conduits.

A first step of the process of the present invention comprises providing a foreshortened, and preferably fibrous, web. The term "foreshortened" web refers to a web which has been reduced in length, i. e., substantially proportionally contracted along its length, in a machine direction. The first step of providing a fibrous web may be preceded by the steps of forming such a web and then foreshortening the web. The fibrous web suitable for the present invention may be made by any papermaking process known in the art, including, but not limited to, a conventional process and a through-air drying process. The present invention also contemplates the use of the web that has been rewetted prior to being foreshortened. The foreshortened web is generally characterized by a plurality of micro-folds running across the web's length, which is known in the art as "crepe." Foreshortening may be accomplished by any method known in the art, for example, by creping, by transferring the web from the first press surface to a slower-moving transfer fabric, or by the combination thereof.

Preferably, the foreshortened web is disposed on a working surface. The preferred working surface has a plurality of fluid-permeable expansion conduits therethrough. One preferred working surface is formed by a belt comprising a (preferably resinous) framework joined to a fluid-permeable reinforcing structure and protruding outwardly from the reinforcing structure, thereby forming the network area. The framework may comprise an essentially continuous and macroscopically monoplanar network area, in which case the plurality of expansion conduits preferably comprises a plurality of discrete orifices, or holes, which are dispersed throughout and encompassed by the continuous network area of the working surface. Alternatively or additionally, the work surface may comprise a plurality of discrete areas formed by discrete protrusions extending from the reinforcing structure, in which case an essentially continuous expansion conduit encompasses the plurality of discrete protrusions.

Preferably, the expansion conduits and/or protrusions are arranged in a pre-selected pattern, and more preferably, the pattern of the arrangement of the expansion conduits and/or protrusions is non-random and repeating. If the patterned working surface comprises discrete areas formed by the individual protrusions, the work surface's discrete areas may have the discrete expansion conduits therethrough, analogous to the discrete expansion conduits in the continuous work surface. The working surface may comprise a surface of a fluid-permeable platen or -- in a preferred continuous process -- a fluid-permeable endless belt or band capable of traveling in a machine direction.

The steps of disposing the foreshortened web on the working surface and moistening the web may be performed either sequentially or simultaneously. If the dry foreshortened web is being first disposed on the working surface, the moisture can subsequently be added to the web disposed on the working surface. Various means may be used for moistening the foreshortened web, such as, for example, spraying the web with water or penetrating the web by steam under pressure. A plurality of jets discharging water onto the selected portions of the web according to a pre-determined pattern may also be used. Preferably, the web, or its selected portions, is/are moistened to have a moisture content from about 95% to about 25%, i. e., the web's preferred fiber-consistency is from about 5% to about 75%. More preferably, the moisture content of the selected portions of the web, after they have been moistened, is from 85% to 35%, i. e., the web's more preferred fiber-consistency is from about 15% to about 65%.

The moisture may be added primarily to the selected portions of the foreshortened web, i. e., those portions which correspond to the expansion conduits of the working surface, and which are not in direct and immediate contact with the working surface. The moisture is added to the selected portions of the web preferably after or simultaneously with the step of disposing the web on the working surface. The moisture added to the web may comprise such functional papermaking additives as softeners and debonders, including, but not limited to, lotions, perfumes, anti-microbial agents, wet-strength resin, etc.

Under the influence of the moisture added, the web's selected portions relax the crepe therein and consequently expand outwardly from the general plane of the web, thus increasing bulk of the web. At the same time, the rest of the web, comprising surface-contacting portions which are in direct and immediate contact with the working surface, retains the crepe therein. The resulting web structure comprises, therefore, at least two distinct regions: a region formed by the web's previously foreshortened portion which has retained the crepe therein, and a region comprising the crepe-relaxed portion having increased (relative to the previously foreshortened portion) caliper. Each of the regions may be substantially continuous, or may comprise a plurality of discrete micro-regions, or a combination thereof. Preferably, the crepe-relaxed portion comprises a plurality of discrete domes outwardly extending from the plane formed by the foreshortened portions of the web. The domes may extend from one side of the web, or from both opposite sides of the web.

One way of retaining crepe in the surface-contacting portions of the foreshortened web comprises adhering the surface-contacting portions to the working surface such as to prevent lateral movement of the surface-contacting portions relative to the working surface with which they are in contact. To accomplish this, the working surface can be treated with an adhesive material, such as, for example, creping adhesive. Alternatively or additionally, the working surface can comprise asperities thereon, preventing the lateral movement of the surface-contacting portions. Other means of creating a sufficient friction between the working surface and the surface-contacting portions of the foreshortened web may be employed to prevent the lateral movement of the surface-contacting portions relative to the working surface.

In the preferred embodiment of the process and the apparatus, a pressing surface, opposite to and facing the working surface, is provided. The pressing surface is a surface adapted to impress the foreshortened web against the working surface. The foreshortened web is constrained, or impressed, between the working and pressing surfaces to the extent necessary to prevent (or contain if desired) expansion of those portions of the web which do not correspond to the expansion conduits. Those portions (defined herein as "surface-contacting portions") retain the crepe therein, while the selected portions of the web are free to expand through the expansion conduits.

The pressing surface may comprise an essentially flat area, or it may have projected areas. The projected areas may comprise continuous network area, or discrete areas, or a combination thereof. Pressing surface may also have expansion conduits therethrough, similar to those of the working surface. The expansion conduits of the pressing surface can correspond to the expansion conduits of the working surface. In the latter instance, the moisture (water and/or steam) can be delivered to and removed from the web using corresponding expansion conduits of the pressing and working surfaces. The latter embodiment provides an additional benefit of allowing the selected portions expand in both opposite directions - through the expansion conduits of the working surface and through the expansion conduits of the pressing surface. In another embodiment, the pressing surface's conduits do not correspond to the working surface's conduits. In this instance some of the selected portions of the web can expand only through the pressing surface's conduits, while the other selected portions can expand only through the working surface's conduits. The last two embodiments of the process and the apparatus allow one to create structured patterned webs.

Preferably, the working surface is associated with a supporting surface such that the working surface having the web thereon is juxtaposed between the pressing surface (contacting the web) and the supporting surface. In the preferred embodiment of the apparatus and the process of the present invention, a temperature differential of at least 50°F is created between the pressing surface and the supporting surface. Preferably, but not necessarily, the pressing surface has a relatively higher temperature, and the supporting surface has a relatively lower temperature. The preferred temperature differential is at least 50°F, and the more preferred temperature differential is at least 100°F. A preferred temperature of the "cold" surface is less than 212°F. The temperature differential drives the moisture added to the web through the web's selected portions thereby relaxing the crepe in the selected portions and causing the selected portions to expand through the expansion conduits. To accumulate the moisture driven through the web, a fluid-permeable fabric is juxtaposed between the "cold" (preferably working) surface and the "hot" (preferably supporting) surface. The fabric should have a void volume sufficient to accumulate the moisture condensing thereinto. This process or any other process known in the art may be used to dry the web.

In one preferred embodiment, the pressing surface comprises a surface of a sintered layer capable of retaining sufficient volume of moisture. The preferred sintered layer comprises metal woven belt capable of containing a sufficient volume of moisture therein and to release the moisture under the influence of the temperature differential. The metal is preferred for its superior heat-transfer properties. When the web and the working surface are impressed between the pressing and supporting surfaces, the moisture contained in the sintered layer moves into and through the web and towards the supporting surface. The crepe in the surface-contacting portions of the web, which are sufficiently contained between the pressing surface and the working surface, is not affected (or affected to a lower degree, if desired) by the water driven through the web from the pressing surface towards the supporting surface. The web's selected areas, which correspond to the expansion conduits of the working surface and/or the pressing surface, are not sufficiently contained between the pressing surface and the working surface, due to the existence of the expansion conduits in both or one of the surfaces. Therefore, the selected portions are not prevented from expanding through the expansion conduits (or prevented to a significantly lower degree relative to the surface-contacting portions). The expanded selected portions of the web form "domes" of a finished product, thereby increasing the bulk or overall caliper of the finished web.

In one of the embodiments of the preferred continuous process of the present invention, each of the pressing surface and the working surface is formed by an endless belt or band traveling in the machine direction. An endless condensation belt (fabric) traveling in the machine direction and capable of receiving a sufficient amount of the condensed moisture is disposed between the supporting surface and the working surface. The moisture which is driven through the selected portions of the web and through the expansion conduits of the working surface condenses into the fabric disposed between the working surface and the supporting surface. A means for collecting and recycling the moisture, well known in the art, may be used in the process of the present invention.

The portions which are impressed between the working surface and the pressing surface may be further densified, if desired. The selected portions of the web corresponding to the expansion conduits are not densified, or densified (if desired) to a lesser degree than the impressed portions are. In the latter instance, a pressure differential may be controlled, on the one hand -- by the distance between the pressing surface and the corresponding working surface, and on the other hand -- by the distance between the pressing surface and a surface restricting the expansion of the selected portions.

In the pressing surface comprising projected areas, some of the projected areas may be registered (either in a knob-to-knob pattern, or in a nested pattern, or in a pattern comprising a combination thereof) with the working surface when the web is impressed between the pressing surface and the working surface. The embodiment of the apparatus is contemplated, in which only some of the projected areas of the pressing surface have corresponding projected areas of the working surface. Thus, some of the selected portions of the web may be partially restrained, in the direction perpendicular to the working surface, to a lesser degree relative to the portions impressed between the working surface and the pressing surface. Consequently, it is believed that the selected portions of the web may comprise in the latter instance sub-portions which are relatively unconstrained in the direction perpendicular to the working surface, and sub-portions which are relatively constrained and may be partially impressed (and therefore possibly densified) by the pressing surface's projected areas corresponding to the expansion conduits of the working surface. Such an arrangement of the working surface and the pressing surface may beneficially produce a web having at least three differential micro-regions: first micro-regions formed by the portions constrained in the direction perpendicular to the working surface and thus substantially retaining the crepe therein; second micro-regions formed by the sub-portions partially-constrained in the direction perpendicular to the working surface and thus having crepe partially relaxed, the second micro-regions partially expanding in the direction perpendicular to the working surface; and the third micro-regions formed by the sub-portions relatively unconstrained in the direction perpendicular to the working surface, having crepe substantially relaxed therein, the third micro-regions expending in the direction perpendicular to the working surface.

The expansion of the selected areas may be assisted by deflecting, under pressure, the moistened selected portions of the web through the expansion conduits. Vacuum or differential pressure can be used as a means for deflecting the selected portions through the expansion conduits. The means for deflecting may also comprise steam or water moving, preferably under pressure, through the selected portions and through the expansion conduits. A combination of steam and water as means for deflecting is also contemplated in the present invention. The pressing surface's projected areas corresponding to the expansion conduits of the working surface can also comprise the means for deflecting the selected portions of the web. In one exemplary embodiment, the projected areas of the pressing surface correspond to the expansion conduits of the working surface and are in contact with the selected portions of the web. When the web is constrained between the pressing surface and the working surface, the projected areas of the pressing surface push the selected portions of the web through the expansion conduits of the working surface, thereby facilitating the expansion of the selected portions.

"Angled" expansion of the selected portions is also contemplated by the present invention. In this instance, the selected portions of the web are caused to expand to form an "angled" position relative to the plane of the belt, i. e., the axes of at least some of the domes formed by the selected portions and the working surface form acute angles therebetween. The working surface may comprise a plurality of protuberances, at least some of which are angled relative to the working surface, i. e., the axes of the protuberances and the working surface form acute angles therebetween. Than, the selected portions of the web, while expanding through the expansion conduits, will take the "angled" position relative to the working surface, and the final web product will have the "angled" continuous domes, i. e., the continuous domes cross-sectional axes of which form acute angles with the general plan of the web.

The web having the crepe relaxed in the selected portions may be re-foreshortened by, for example, adhering the crepe-relaxed and expanded selected portions of the web to the creping surface and then creping therefrom with a doctor blade.

### BRIEF DESCRIPTION OF THE DRAWINGS

FIG. 1 is a schematic and simplified side elevational view of the apparatus of the present invention, showing a web disposed on a working surface.
FIG. 2 is a view similar to one shown in FIG. 1, and showing the web being impressed between the working surface and a pressing surface.
FIG. 3 is a schematic and simplified side elevational view of another embodiment of the apparatus of the present invention, having a pressing surface comprising extending projected areas.
FIG. 4 is a schematic and simplified side elevational view of still another embodiment of the apparatus of the present invention, having a pressing surface comprising extending projected areas and expansion conduits.
FIG. 5 is a schematic and simplified side elevational view of another embodiment of the apparatus of the present invention, showing the pressing surface comprising a sintered layer.
FIG. 5A is a schematic and simplified side elevational view of still another embodiment of the apparatus comprising two mutually opposite surfaces having corresponding expansion conduits therethrough.
FIG. 6 is a schematic plan view of one embodiment of the working surface comprising a plurality of discrete conduits, taken along lines 6-6 of FIG. 1.
FIG. 7 is a schematic plan view of another embodiment of the working surface comprising a continuous conduit, taken along lines 7-7 of FIG. 3.
FIG. 8 is a schematic and simplified side elevational view of another embodiment of the apparatus of the present invention, showing both the pressing surface and the working surface having the expansion conduits therethrough, the expansion conduits of the working surface partially corresponding to the expansion conduits of the pressing surface.

### DETAILED DESCRIPTION OF THE INVENTION

The present invention provides a process and an apparatus for increasing bulk of a foreshortened web by causing selected portions of the foreshortened web to relax crepe, thereby expanding outwardly from one or both opposite sides of the web.

A first step of the process of the present invention comprises providing a foreshortened, and preferably fibrous, web. As used herein the term "fibrous web" or simply "web" designates a macroscopically planar substrate comprising cellulosic fibers, synthetic fibers, or any combination thereof. The first step of providing a web 60 may be preceded by the steps of forming such a web and then foreshortening the web. One skilled in the art will readily recognize that forming the web 60 may include the steps of providing a plurality of papermaking fibers. Suitable fibers comprising the web **60** may include recycled, or secondary, papermaking fibers, as well as virgin papermaking fibers. Such fibers may comprise hardwood fibers, softwood fibers, and non-wood fibers.

In a typical continuous papermaking process, the plurality of fibers are preferably suspended in a liquid carrier. More preferably, the plurality of fibers comprises an aqueous dispersion. An equipment for preparing the aqueous dispersion of fibers is well-known in the art and is therefore not illustrated herein. The aqueous dispersion of fibers may be provided to a headbox or headboxes. The headbox(es) and the equipment for preparing the aqueous dispersion of fibers are typically of the type disclosed in U.S. Patent No. 3,994,771, issued to Morgan and Rich on November 30, 1976. The preparation of the aqueous dispersion of the papermaking fibers and exemplary characteristics of such an aqueous dispersion are described in greater detail in U.S. Patent 4,529,480, which patent is incorporated by reference herein. The fibrous web suitable for the present invention may be made by any papermaking process known in the art, including, but not limited to, a conventional process and a through-air drying process. The present invention also contemplates the use of the web 60 that has been rewetted. Rewetting of a previously-manufactured dry web may be used for creating three-dimensional web structures by, for example, embossing the rewetted web and than drying the embossed web.

As used herein, the term "foreshortened" web refers to a web which has been substantially proportionally contracted along its length, i. e., in a machine direction. In the papermaking, the machine direction, or MD, indicates that direction which is parallel to and has the same direction as the flow of the web through a papermaking equipment. The cross-machine direction, or CD, is perpendicular to the machine direction and parallel to the general plane of the web.

The foreshortened web is generally characterized by a plurality of micro-folds running across the web's length. Such micro-folds are typically known in the art as "crepe." Foreshortening may be accomplished by any method known in the art, for example, by creping, by transferring the web from the first press surface to a slower moving transfer fabric, or by the combination thereof. As used herein, the web which has been foreshortened has crepe therein, regardless of the method of foreshortening.

Creping is usually performed with a creping doctor blade juxtaposed with the creping surface having the web adhered thereto. Creping may be accomplished according to commonly assigned U. S. Patent 4,919,756, issued on April 24, 1992 to Sawdai, the disclosure of which is incorporated herein by reference. A conventional creping blade is positioned against the creping surface so as to create an impact angle between the blade and the creping surface, wherein the impact angle ranges from about 70 degrees to about 90 degrees. A creping adhesive may be applied directly to the creping surface. Creping adhesives comprising polyvinyl alcohol, animal-based protein glues, or mixtures thereof, well known in the art, may be utilized. The commonly-assigned U.S. Patent 3,926,716 issued to Bates on Dec. 16, 1975, teaches a polyvinyl alcohol creping adhesive. The U.S. Patent 4,501,640 issued to Soerens on Feb. 26, 1985; U.S. Patent 5,187,219 issued to Furman, Jr. on Feb. 16, 1993; U.S. Patent 5,494,554 issued to Edwards et al. on Feb. 27, 1996 describe various types of creping adhesives. Optionally, various plasticizers may be used in conjunction with the creping adhesive. For example, the plasticizer commercially sold as CREPETROL R 6390 is available from Hercules Incorporated of Wilmington, DE.

Foreshortening comprises a process commonly described as a "microcontraction." Microcontraction includes transferring the web from one moving surface (typically a foraminous member or a papermaking belt) to another, a slower-moving surface (typically a transfer belt). U. S. Patent 4,440,597, commonly assigned; describes in detail a "wet-microcontraction." Briefly, wet-microcontraction involves transferring the web having a low fiber-consistency from a first member (such as a foraminous member) to a second member (such as a loop of open-weave fabric) moving slower than the first member. According to U.S. Patent 4,440,597, the preferred consistency of the web prior to the transfer is from about 10% to about 30% fibers by weight, and the most preferred consistency is from about 10% to about 15%. Commonly-assigned patent application entitled "Process and Apparatus For Making Foreshortened Cellulosic Structure," filed in the names of Carol A. McLaughlin et al. on 12/19/97 (P&G Case # 6966), is incorporated by reference herein.

The next step in the process of the present invention may comprise providing a working surface **20** designed to receive the foreshortened fibrous web **60.** FIGs. **1-7** show various embodiments of the working surface **20.** Regardless of the embodiment, the preferred working surface **20** has a plurality of fluid-permeable micro-regions, or expansion conduits, **25** therethrough. As used herein, the term "fluid-pervious" refers to the capability of the expansion conduits **25** to have a fluid, such as liquid (water) or gas (air or steam), transmitted through the conduits **25** without significant obstruction. The conduits **25** are termed "expansion conduits" because they provide void areas through which selected portions of the web can expand outwardly, as will be explained in greater detail below. The preferred expansion conduits **25** comprise unobstructed orifices, or holes, through the working surface **20**. Preferably, the expansion conduits **25** are arranged in a pre-selected pattern, and more preferably, the pattern of their arrangement is non-random and repeating throughout the working surface.

One preferred working surface **20** is formed by a belt comprising a framework **21** joined to a reinforcing structure **23,** as shown in FIGs. **1-3.** Preferably, the framework **21** is resinous. The framework **21** protrudes outwardly from the reinforcing structure **23**, thereby forming the network area **22**, as best shown in FIGs. **1** and **6.** This type of belt is described in several commonly-assigned U.S. Patents incorporated by reference herein and referred to above. In the embodiment shown in FIGs. **1**, **6**, and **2**, the network **22** is essentially continuous and macroscopically monoplanar, and the plurality of fluid-permeable conduits **25** comprises a plurality of discrete orifices, or holes, which are dispersed throughout and encompassed by the essentially continuous network **22**. As used herein, the term "essentially continuous" indicates that interruptions in absolute geometrical continuity, while are not preferred, may be tolerable -- as long as these interruptions do not adversely affect the performance of the framework **21** and network **22**. It should also be carefully noted that embodiments (not shown) are possible in which interruptions in the absolute continuity of the framework **21** (and thus network **22)** are intended as part of the overall design of the working surface **20**.

Preferably, the conduits **25** are arranged in a pre-selected pattern throughout the network **22**, and more preferably, the pattern of the arrangement of the conduits **25** is non-random and repeating, such as, for example, a continuously-reticulated pattern, best shown in FIG. **6**. The belt having a continuous network **22** and discrete fluid-permeable expansion conduits **25** is primarily disclosed in the commonly assigned.

The patterned working surface **20** may comprise discrete areas, alternatively or in addition to the continuous network **22.** FIGs. **3** and **7** show the working surface **20** comprising a plurality of discrete areas formed by discrete protrusions **27** outwardly extending from the reinforcing structure **23** and separated from one another by an area of essentially continuous expansion conduits **25**. The discrete areas formed by the individual protrusions may have the discrete expansion conduits therethrough, similar to the discrete expansion conduits described above in the context of the continuous working area. The belt having the framework **21** comprising the discrete protrusions is primarily disclosed in the commonly assigned and U.S. Patent 4,245,025 issued Sep. 14, 1993 to Trokhan et al. and U.S. Patent 5,527,428 issued June 18, 1996 to Trokhan et al. Also, the papermaking belt having the discrete protuberances raised above the plane of the fabric may be made according to the European Patent Application 95105513.6, Publication No. 0 677 612 A2, filed 12.04.95, inventor Wendt et al.

The working surface **20** may comprise a fluid-permeable platen, or -- in a preferred continuous process -- a fluid-permeable endless belt or band 28, as schematically shown in FIG. **5**. The endless belt or band **28** is designed to continuously travel in the machine direction. Fluid-permeability of the band **28** may be achieved by perforating (preferably, according to a pre-determined pattern) the band **28** throughout its thickness or by other conventional means -- to provide expansion conduits **25.** Preferably, the band **28** is juxtaposed with a fluid-permeable fabric **50** (FIGs. **4** and **5).** The fabric **50** should preferably have a sufficient amount of void volume to be able to receive moisture driven into the fabric **50** from the web **60**, as will be explained in greater detail below. The fabric **50** can be woven or non-woven. One preferred fabric comprises Spiral Weave, Duraflex Belt made by Albany International, Engineered Fabrics of Portland, TN.

The next two steps in the process of the present invention comprise disposing the foreshortened web **60** on the working surface **20** and moistening the web **60.** These steps may be performed sequentially or simultaneously. If the dry foreshortened web **60** is being first disposed on the working surface **20**, the moisture can subsequently be added to the web **60** associated with the working surface **20**. If the foreshortened web **60** is being first moistened and then disposed on the working surface **20**, wet transfer may be used in the process of the present invention for the step of depositing the web **60** on the working surface **20**. As one skilled in the art will recognize, wet transfer comprises transferring the wet web from one carrier (a foraminous member or a belt) to another carrier using vacuum or differential pressure.

Various means may be used for moistening the foreshortened web **60**. For example, the foreshortened web **60** can be sprayed with water or moistened by steam. Preferably, the web **60** is moistened to have a moisture content from about 95% to about 25%. More preferably, the moisture content of the web **60**, after it has been moistened, is from about 80% to about 40%.

According to the present invention, the entire web **60** can be moistened to have the necessary moisture content. Alternatively, moisture may be added primarily to selected portions **62** of the web **60.** As used herein, the "selected portions" **62** of the web **60** are those portions which correspond to the expansion conduits **25** of the working surface **20** when the web is disposed on the working surface **20**. Preferably, the selected portions **62** are not in direct and immediate contact with the working surface **20**, due to the existence of the expansion conduits **25**. In the instance when the moisture is added primarily to the selected portions **62** of the web **60**, it is preferred that the step of moistening the foreshortened web **60** be performed after or simultaneously with the step of disposing the web **60** on the working surface **20**.

The moisture added to the web **60** may comprise various functional papermaking additives, such as softeners and debonders. Examples include, but are not limited to: nonionic surfactant described in U.S. Patent 5,527,560, issued June 18, 1996 to Fereshtehkhou et al.; a softening composition comprising quaternary ammonium compound, polysiloxane compound, and binder materials described in commonly-assigned U.S. Patent 5,573,753, issued November 12, 1996 to Ampulski et al.; a water-soluble polyhydroxy compound described in commonly-assigned U.S. Patent 5,624,532, issued April 29, 1997 to Phan et al.; a debonder described in Canadian Patent 2,118,529, issued February 2, 1996 to Edwards et al.; softening agent described in U.S. Patent 5,716,498, issued February 10, 1998 to Jenny et al.; a cationic nitrogenous softener/debonder described in U.S. Patent 5,695,607, issued December 9, 1997 to Awofeso et al.; softeners/debonders described in U.S. Patent 5,552,020, issued September 3, 1996 to Schroeder et al.; a cationic silicone described in U.S. Patent 5,591,306, issued January 7, 1997 to Kaun et al.; and others. Other functional additives, such as lotions, emulsions, perfumes, anti-microbial and anti-bacterial agents, and wet-strength resin may also be included into the moisture.

According to the present invention, the moisture added to the web **60** or to the web's selected portions **62** relaxes the crepe in the selected portions **62**. Consequently, the selected portions **62** expand outwardly from the general plane of the web **60**, thus increasing bulk of the web **60**. Preferably, the selected portions **62** expand through the expansion conduits **25** of the working surface **20**. At the same time, in accordance with the present invention, the rest of the web **60** retains the crepe therein. As used herein, the rest of the web which retains the crepe is defined as comprising "surface-contacting portions" **61** of the web **60**, for the surface-contacting portions **61** are in direct and immediate contact with the working surface **20**, in contrast with the selected portions **62** corresponding to the expansion conduits **25**.

In the embodiment in which the moisture is added only to the web's selected portion **62**, the surface-contacting portions **61** retain the crepe primarily by virtue of not being moistened. Additionally, the working surface **20** may be treated to enhance friction between the working surface **20** and the surface-contacting portions **61,** which friction should preferably be sufficient to prevent the surface-contacting portions **61** from laterally moving relative to the working surface **20**. The friction between the working surface **20** and the surface-contacting portions **61** may be enhanced by, for example, providing the working surface **20** with asperities thereon, designed to mechanically engage the surface-contacting portions **61** such as to prevent or restrict their lateral movement. Alternatively or additionally, the working surface can be treated with a suitable adhesive, to temporarily adhere the surface-contacting portions **61** to the working surface **20**. Neither the asperities nor the adhesive treatment are illustrated in the drawings, for one skilled in the art will easily visualize both embodiments. Other means of creating a sufficient friction between the working surface **20** and the surface-contacting portions **61** of the web **60** may be employed in the apparatus of the present invention to prevent the lateral movement of the surface-contacting portions **61** relative to the working surface **20**.

After the crepe has relaxed in the selected portions **62** under the influence of moisture, while the rest of the web **60** retains the crepe, the web **60** comprises at least two distinct regions: a region formed by the web's previously foreshortened portion which has retained the crepe therein (i. e., comprising the surface-contacting portions **61**), and a region formed by the crepe-relaxed portions (i. e., comprising the selected portions **62)** extending outwardly from the general plane of the web **60** and thereby preferably having increased caliper, relative to the surface-contacting portions **61**. Each of the regions may be substantially continuous, or comprising a plurality of discrete micro-regions, or a combination thereof, depending on the design of the working surface **20**, as has been discussed above. Preferably, in the final product the crepe-relaxed selected portions **62** comprise a plurality of discrete domes outwardly extending from the plane formed by the foreshortened portions of the web **60**. The domes may extend from one side of the web **20** (FIGs. **2-5**), or from both opposite sides of the web **20** (FIGs. **5A** and **8**).

Optionally, the moistened selected portions **62** of the web **60** may be subjected to deflection into the expansion conduits **25** of the working surface **20** to facilitate expansion of the selected portions **62** of the web **60** through the expansion conduits **25** of the working surface **20**. A variety of deflecting means may be used in the process and the apparatus **10** of the present invention. One skilled in the art will recognize that vacuum pressure or pressure differential may be used as deflecting means. The deflecting means may also comprise steam or water moving, preferably under pressure, through the selected portions **62** and through the expansion conduits **25** of the working surface **20**. A combination of steam and water as deflecting means is also contemplated by the present invention.

One preferred embodiment of the apparatus **10** comprises a pressing surface **30**. The pressing surface **30** is a surface designed to constrain, or impress, the web **60** against the working surface **20**. The pressing surface **30** is opposite to the working surface **20** and preferably substantially parallel to the working surface **20**. Although the drawings show the pressing surface **30** and the working surface **20** as substantially planar surfaces, it should be appreciated that both the pressing and working surfaces **30**, **20** can be curved, or have other non-planar configuration, as long as they are capable of receiving and constraining the web **60** therebetween.

FIGs. **1-8** show several exemplary embodiments of the pressing surface **30.** In FIGs. **1** and **2,** the pressing surface **30** comprises an essentially flat and unpattemed area. In FIGs. **3** and **4,** the pressing surface **30** comprises projected areas **31**, preferably having a pre-determined pattern. The projected areas **31** may comprise a substantially continuous or ― alternatively ― discrete area, as has been explained above in the context of the network **22** of the working surface **20**. The combination of continuous areas and discrete areas of the pressing surface **30** is also contemplated in the present invention. FIGs. **3** and **4** show that at least some of the projected areas **31** of the pressing surface correspond to the expansion conduits **25** of the working surface **20**. In these two embodiments, the deflecting means comprises the projected areas **31** of the pressing surface **30**, corresponding to the expansion conduits **25** of the working surface **20**. The projected areas **31** facilitate the expansion of the selected portions **62** through the conduits **25**.

As shown in FIGs. **4** and **8,** the pressing surface **30,** whether flat or having the projected areas **31**, may comprise expansion conduits **35**, similar to those of the working surface **20.** FIG. **4** shows the expansion conduits **35** which correspond to the projected areas **31**, and FIG. **8** shows the conduits **35** which do not correspond to the projected areas **31.** In both instances, however, when the web **60** is constrained between the pressing surface **30** and the working surface **20**, at least some of the expansion conduits **35** of the pressing surface **30** correspond to the expansion conduits **25** of the working surface **20**, as shown in FIGs. **4** and **8.** Of course an embodiment is possible in which none of the expansion conduits **35** of the pressing surface **30** correspond to the expansion conduits **25** of the working surface **20** (not shown).

FIG. **5** shows an embodiment of the pressing surface **30** comprising a surface of a sintered layer **40** capable of retaining sufficient volume of moisture. The sintered layer **40** is one preferred means for moistening the web **60.** The sintered layer **40** can be made from any suitable material. One preferred material for the sintered layer **40** is sintered stainless steel having pores of about 40 micro-meter (µm) in diameter, made by Mott Corporation, 84 Spring Lane Farmington, CT 06032-3159. Preferably, the sintered layer **40** is capable of retaining a moisture therein in the amount sufficient to moisten the web 60 to the required consistencylmoisture content as defined herein.

The apparatus **10** of the present invention preferably further comprises a supporting surface **24.** The supporting surface **24,** shown in FIGs. **4, 5,** and **8** is a surface designed such that the working surface **20** is capable of being interposed between the supporting surface **24** and the pressing surface **30**, the working surface **20** facing the pressing surface **30**. Preferably, the supporting surface **24** does not directly contact the working surface **20**. That is, as shown in FIGs. **4** and **5**, there is a distance D between the working surface **20** and the supporting surface **24**. Preferably, the supporting surface **24** is associated with the working surface **20** through the fabric **50,** as shown in FIGs. **4** and **5.** In the embodiment of the apparatus **10** and the process of the present invention, comprising the supporting surface **24**, the process step of constraining the foreshortened web **60** between the working surface **20** and the pressing surface **30** comprises impressing the working surface **20** with the associated web **60** thereon between the pressing surface **30** and the supporting surface **24.**

In one preferred embodiment of the process of the present invention, schematically illustrated in FIG. **5,** the dry foreshortened web **60** is first disposed on the working surface **20** by any conventional means. Then, the foreshortened web **60** disposed on the working surface **20** is contacted by the working surface **20** such that the web **60** is constrained between the pressing surface **30** and the pressing surface **30** comprising the sintered layer **40**. When the web **60** is thus contacted by the sintered layer **40**, the web **60** starts receiving moisture from the sintered layer **40** at one of the web's sides. A pressure may be applied to facilitate moistening of the web **60** by the sintered layer **40**.

In accordance with the preferred embodiment of the present invention, a temperature differential is created between the pressing surface **30** and the working surface **20**. The temperature differential should be sufficient to cause the moisture added to at least the selected portions **62** of the web **60** to move through the selected portions **62** in the direction from one of the surfaces **30, 20** to the other **20, 30.** Preferably, the temperature differential between the pressing surface **30** and the working surface **20** is provided by heating the pressing surface **30** to a temperature T1, and maintaining the supporting surface **24** at a temperature T2 sufficiently lower than T1. Thus, the temperature differential between the pressing surface **30** and the working surface **20** is preferably provided by creating the temperature differential between the pressing surface **30** and the supporting surface **24.** In the drawings, the preferred arrangement is illustrated, in which the web's side which contacts the pressing surface **30** is first moistened, and the moisture is driven under the temperature differential from the pressing surface **30** to the working surface **20**, and further through the expansion conduits **25** of the working surface **20** into the fabric **50**. However, one skilled in the art should appreciate that the direction of the movement of the moisture through the web **60** could be reversed, provided the temperature of the working surface **20** is sufficiently greater relative to the temperature of the pressing surface **30**. It should also be appreciated that, as used herein, the terms "pressing surface" and "working surface" are relative terms, and the expansion conduits may be provided in both or either one of the pressing surface **30** and the working surface **20**. Consequently, the selected portions **62** of the web **60** can expand through the conduits of both or either one of the pressing surface **30** and working surface **20.**

In the preferred embodiment, the pressing surface **30** is heated to have the temperature T1 higher than the temperature T2 of the supporting surface **24.** In FIG. **4,** the temperature differential ΔT between the pressing surface **20** and the supporting surface **24** causes the moisture contained in the sintered layer **40** move into and through the web **60** and towards the supporting surface **24**. Because the surface-contacting portions **61** of the web **60** are sufficiently constrained between the pressing surface **30** and the working surface **20**, the crepe in the surface-contacting portions **61** is not affected (or, if desired, affected to a lower degree) by the moisture driven through the web **60** from the pressing surface **30** towards the supporting surface **20**. However, due to the existence of the expansion conduits **25** in the working surface **20**, the selected areas **62**, which correspond to the expansion conduits **25**, are not constrained or constrained, if at all, only at one side associated with the pressing surface **30**, as FIG. **5** shows. Therefore, the selected portions **62** are relatively free to expand towards the supporting surface **24**. The preferred temperature differential ΔT between the pressing surface **30** and the supporting surface **24** is at least 50°F, and the more preferred temperature differential ΔT is at least 100°F. The temperature T2 of the "cool" surface (i. e., the supporting surface **24** in FIGs. 4, 5, and 8) is preferably less than 212°F.

FIG. **5A** shows an embodiment in which the selected portions **62** are relatively unconstrained at both sides of the web **60,** for in FIG. **5A** the expansion conduits **25** of the working surface **20** correspond to the expansion conduits **35** of the pressing surface **30.** It should also be understood that while FIG. **5A** shows the embodiment in which the same selected portion **62** expands outwardly at both mutually opposite sides of the portion **62**, the embodiment is possible (and may even be preferred) in which some of the selected portions **62** expand outwardly at one side of the web **60**, while the other selected portions **62** expand at the other (opposite) side of the web **60**. An embodiment is also possible in which the selected portions **62** partially expand outwardly at both mutually opposite sides of the web **60,** as shown in FIG. **8**, i. e., only part of the selected portion(s) **62** expands at both sides of the web **60**. In FIG. **8**, the conduits **35** of the pressing surface **30** partially correspond to the conduits **25** of the working surface **20**.

Preferably, the selected portions **62** are free to expand through the expansion conduits **25** and **35**. It is believed that the moisture moving through the selected portions **62** and through the expansion conduits **25** in the direction towards the supporting surface **24** facilitates expansion of the selected portions **62** through the expansion conduits **25,** thereby relaxing the crepe in the selected portions **62** of the web **60.** As the moistened selected portions **62** of the web **60** expand through the expansion conduits **25** and/or **35,** the caliper of the selected portions **60** increases, thereby increasing the overall bulk of the web **60.** In the finished web product (not shown), the selected portions **62** have a pattern which in plan view is essentially similar to the pattern of the working surface **20** including the expansion conduits **25** and/or **35.** The preferred continuous and still foreshortened area comprising the surface-contacting portions **61** provides strength, while the discrete domes comprising crepe-relaxed selected portions **62** generate bulk, and thus are believed to improve softness and absorbency of the final web product. Additional densification of the surface-contacting portions 61 may provide further improvement of the finished web product's strength.

While not preferred, the steam moving under pressure through the web's selected portions **62** may be used in the present invention even without the use of the pressing surface **30** and the supporting surface **24**, and without the assistance of the temperature differential ΔT between the pressing surface **30** and the supporting surface **24**. One skilled in the art may easily visualize an embodiment (not shown) in which steam is forced to penetrate under pressure the selected portions **62** and move through the expansion conduits **25**, thereby causing the crepe in the selected portions **62** to relax and the selected portions **62** to expand. In the latter embodiment, the steam preferably condenses into the fabric **50** and is recycled.

FIGs. **4** and **5** show preferred embodiments of the apparatus **10** of the present invention, comprising two opposite members: a pressing member **36** having the pressing surface **30**, and a supporting member **26**, having the supporting surface **24**. In the preferred continuous process of the present invention, each of the pressing member **36** and the supporting member **26** comprises an endless belt or band traveling in the machine direction. In FIG. **5**, the pressing member **36** comprises the sintered layer **40**; and the supporting member **26** is associated with the moisture-receiving fabric **50**, also comprising an endless belt. Preferably, the moisture which is driven through the selected portions **62** of the web **60** through the expansion conduits **25** of the working surface **20** condenses into the fabric **50** disposed between the working surface **20** and the supporting surface **24.** Preferably, a means for collecting and recycling the moisture, well known in the art, is used in the process of the present invention.

As shown in FIGs. **2-5,** the selected portions **62** of the web **60** correspond to the expansion conduits **25** of the working surface **20,** and the surface-contacting portions **61** of the web **60** correspond to and are in contact with the working surface **20**. In FIGs. **2-5**, the surface-contacting portions **61** are constrained between the working surface **20** and the pressing surface **30**. As has been explained above, the pressure should be sufficient to effectively constrain the portions **61** in the direction perpendicular to the working surface **20** so as to retain the crepe existing in the surface-contacting portions **61.** However, if desired, the pressure may be applied in excess of that which is necessary to retain the crepe in the surface-contacting portions **61**. In the latter instance, the surface-contacting portions **61** may be densified, while the selected portions **62**, corresponding to the expansion conduits **25**, are not densified, or ― if desired ― densified to a lesser degree than the surface-contacting portions **61** are. By densifying the foreshortened surface-contacting portions **61**, one might achieve further improvement in the web's strength. One skilled in the art will appreciate that the degree of relative densification of the surface-contacting portions **61** and the selected portions **62** may depend upon the applied pressure and a relative geometry of the working surface **20** and the pressing surface **30**. If desired, the selected portions **62** of the web **60** may also be constrained in the direction perpendicular to the working surface **20**. For example, the selected portions **62** may be impressed between the pressing surface **30** and the fabric **50**, as shown in FIG. **4**. In the latter instance, both the surface-contacting portions **61** and the selected portions **62** of the web **60** may be densified, but to a different degree. The pressure differential between the pressure applied to the surface-contacting portions **61** and the pressure applied to the selected portions **62** may be controlled, on the one hand -- by the distance between the pressing surface **30** and the corresponding working surface **20**, and on the other hand ― by the distance between the pressing surface **30** and a surface restricting the expansion of the portions **62,** i. e., the surface of the reinforcing structure **23** in FIG. **3**, or the surface of the fabric **50** in FIG. **4.**

FIGs. **3** and **4** show two exemplary embodiments of the working surface **20** superimposed with the pressing surface **30.** In FIG. **3,** the pressing surface **30** comprises the projected areas **31.** Some of the projected areas **31**, i. e., the projected areas designated as **31b,** correspond to (or registered with) the working surface **20.** Other projected areas **31**, i. e.., the projected areas designated as **31a,** correspond to (or registered with) the expansion conduits **25** of the working surface **20.** While the embodiment of the working surface **20** shown in FIGs. **3** and **7** comprises discrete protuberances **27** encompassed by the continuous expansion conduit **25**, it is to be understood that the projected areas of both the working surface **20** and the pressing surface **30** may (and preferably do) comprise the continuous network **22** described therein above and best shown in FIG. **6**. (One skilled in the art will appreciate that the schematic side elevational view shown in FIG. **3** is equally applicable to the network **22** comprising both the continuous pattern shown in FIG. **6**, and the discrete pattern shown in FIG. **7**.)

It should be carefully noted that in FIG. **3,** some of the projected areas **31,** i. e., the projected areas **31a,** of the pressing surface **30** have no corresponding protuberances **27** of the working surface **20,** hence no corresponding working surface **20.** Still, the selected portions **62** of the web **60** may be partially restrained between the projected areas **31a** and the reinforcing structure **23.** The selected portions **62** are constrained to a lesser degree relative to the selected portions **61.** Because the projected areas **31a** correspond to the expansion conduits **25** of the working surface **20,** under the temperature differential ΔT the moisture travels from the projected areas **31a** through the web **60**, as has been described above. In the embodiment shown in FIG. 3, the pressure caused by the projected areas **31a** partially impressing the selected portions **62** against the reinforcing structure **23** is less than the pressure caused by the projected areas **31b** impressing the surface-contacting portions **61** against the working surface **20.** Therefore, it is believed that in the embodiment schematically shown in FIG. **3** the selected portions **62** comprise sub-portions **62a** which are relatively unrestrained in the direction perpendicular to the working surface **20**, and sub-portions **62b** which are restrained and may be partially impressed by the projected areas **31a** corresponding to the expansion conduits **25** of the working surface **20.** Without wishing to be limited by theory, Applicants believe that this principal arrangement of the working surface **20** and the pressing surface **30** may beneficially produce a web having at least three differential micro-regions: a first micro-region formed by the surface-contacting portions **61** constrained in the direction perpendicular to the working surface **20** and thus substantially retaining crepe therein; a second micro-region formed by the sub-portions **62b** partially-constrained and partially expanding in the direction perpendicular to the working surface **20** and thus having the crepe partially relaxed therein; and a third micro-region formed by the sub-portions **62a** relatively unconstrained in the direction perpendicular to the working surface **20** and having crepe substantially relaxed therein, the sub-portions **62a** of the third micro-region expending in the direction perpendicular to the working surface **20.**

In FIG. **4,** showing another exemplary embodiment of the apparatus **10** of the present invention, the projected areas **31** of the pressing surface **30** are registered with the conduits **25** of the working surface **20** such that when the web **60** is constrained between the pressing surface **30** and the working surface **20,** the projected areas **31** facilitate deflection of the selected portions **62** into the expansion conduits **25** of the working surface **20**. In FIG. **4,** the projected areas **31** of the pressing surface **30** correspond to the expansion conduits **25** of the working surface **20** and are in contact with the selected portions **62** of the web **60.** When the web **60** is impressed, the projected areas **31** push, by contact, the selected portions **62** into the conduits **25,** thereby causing the selected portions **62** to expand, as shown in FIG. **4.**

While FIGs. **2-5** show the selected portions **62** of the web **60** expending substantially perpendicular to the working surface **20** and to the general plane of the web **60**, "angled" expansion of the selected portions **62** is also contemplated by the present invention. Two commonly assigned patent applications, Serial No. 08/858,662 and Serial No. 08/858,661, both entitled "Cellulosic Web, Method and Apparatus for Making the Same Using Papermaking Belt Having Angled Cross-Sectional Structure, and Method of Making the Belt". The former application discloses a papermaking belt comprising a continuous resinous framework joined to a reinforcing structure and having a plurality of discrete conduits therein, at least some of the conduits having an "angled" position relative to the plane of the belt, i. e., the axes of the conduits and the surface of the belt form acute angles therebetween. The latter application discloses the belt having a plurality of resinous protuberances joined to the reinforcing structure, and a continuous conduit, at least some of the protuberances being angled relative to the surface of the belt, i. e., the axes of the protuberances and the surface of the belt form acute angles therebetween. These embodiments are not illustrated herein, for in view of the two commonly-assigned patent application cited herein above one skilled in the art will be able to easily visualize the "angled" expansion of the selected portions **62** of the web **60**.

The web **60**, after having been subjected to the process of the present invention, may be re-foreshortened, if desired. As used herein, the term "re-foreshortening" refers to the process of foreshortening the web which has already been at least partially foreshortened. For example, the web **60**, comprising the previously-foreshortened portions **61** and the expanded selected portions **62**, may be adhered to a creping surface and then creped therefrom with a creping blade.

By way of illustration, and not by way of limitation, the following examples are presented. A conventionally-made, creped paper web, having basis weight of about 11 pounds per 3000 square feet, and the caliper of 6.0 mil, was crepe-relaxed according to the present invention and then tested. The following TABLE illustrates results of the testing.

**TABLE**

| Test | Pressure (psi) | Fiber-Consistency (%) | Resulting Caliper (mils) | Change in Caliper (%) |
|---|---|---|---|---|
| Base | N/A | about 95 | 6.0 | N/A |
| I | 55 | 20 | 8.9 | +48.3 |
| II | 55 | about 95 | 5.3 | ―13.2 |
| III | 55 | 20 | 8.2 | +36.6 |
| IV | 55 | about 95 | 5.2 | ―15.4 |

For comparison, a base sample of the dry web having caliper of 6.0 mils, which was not subjected to the process of the present invention, is shown in the first line of the Table.

Tests I and II were conducted using the apparatus **10** of the present invention, principally illustrated in FIG. **5.** More specifically, this apparatus **10** comprises the working surface **20** formed by the surface of a 6"×6" platen **28** having a plurality of expansion conduits **25** therein, and the pressing surface **30** formed by the surface of the sintered layer **40**. The conduits **25** are distributed throughout the working surface **20** in a staggered pattern such that the platen **28** has 40% open area (i. e., conduits **25** comprise 40% of the entire platen's surface). The platen **28** is made of a perforated metal, 14 gauge AL. Each of the conduits **25** is an aperture having 0.125" diameter. The sintered layer **40** is formed by a
6"×10"×0.078" Sintered Stainless Steel, having 40µm pore size, made by Mott Corporation and referred to herein above. The platen **28** is adjacent to the condensation fabric **50** formed by 6"×6" portion of the Spiral Weave, Duraflex Belt, made by Albany International, Inc., which was referenced herein above.

Tests III and IV were conducted using the apparatus **10,** schematically shown in FIG. **5A.** This apparatus **10** comprises two mutually opposite 6"×6" platens **28**, described in the previous paragraph. The platens **28** are interposed such that their respective conduits **25** and **35** correspond, as shown in FIG. **5A**. The sintered layer **40** and the fabric **50** are identical to those described in the previous paragraph.

In all tests I-IV, a press (not shown) was used to cause the pressing member **36** and the supporting member **26** to move towards each other and to impress the working surface **20** with the associated web **60** therebetween. The press used is Carver Laboratory Press, Model "C," made by Carver, Inc., of Indiana (1569 Morris street, Wabash, IN 46992-0544). The press is equipped with 6"×6" Electric Heating Platens, Catalog No. 2101, available from Carver, Inc. In all I-IV tests, the web **60** was interposed between the working surface **20** and the pressing surface **30**, the web **60** was at least partially moistened and impressed between the pressing and working surfaces **30**, **20** at pressure of **55** psi (cylinder pressure) for 7 minutes. Then, the caliper of the selected portions of the dried web **60** (having fiber-consistency of about 95%) was measured.

In Test I, the entire sample of the web **60** was moistened to have fiber-consistency of about 20%. As TABLE shows, the caliper of the web **60** increased to 8.9 mils, i. e., by more than 48% relative to the base sample's caliper of 6.0 mils. For comparison, in Test II, a dry (about 95% fiber-consistency) sample of the web **60** was impressed under the same pressure; the resulting caliper was only 5.3 mils.

In Test III, only the selected portions **62,** corresponding to the expansion conduits **25** and **35** were moistened to have fiber-consistency of about 20%. The resulting caliper of the selected portions **62** was 8.2 mils, i. e., increased by more than 36%, relative to the base sample's caliper of 6.0 mil. In Test IV, the dry (about 95% fiber-consistency) sample of the web, after having been impressed at the pressure of 55 psi, had 5.2 mils caliper.

Caliper of the selected portions **62** of web **60** was measured as the thickness of the "preconditioned" selected portions **62** when subjected to a compressive load of 15 gram per square centimeter (g/cm²), or 95 gram per square inch (g/in²), with a presser foot having diameter of 2 inches (5.08 cm). The term "preconditioned" means a web subjected to a temperature of (23±1)°C, and a relative humidity of (50±2)% for 24 hours, according to a TAPPI Method # T4020M-88. The caliper was measured with a Thwing-Albert model 89-11 thickness tester made by Thwing-Albert Co. of Philadelphia, PA.

## Claims

1. A process for increasing bulk of a foreshortened web, the process comprising steps of:
(a) providing a foreshortened web comprising crepe and having a general plane;
(b) adding moisture to at least selected portions of the foreshortened web, thereby causing relaxation of the crepe in the selected portions of the web and expansion of the selected portions of the web outwardly from the general plane of the web; and
(c) retaining the crepe in the rest of the web.

2. The process according to Claim 1, further comprising the steps of
providing two mutually opposite surfaces designed to receive the foreshortened web therebetween, at least one of the surfaces having a plurality of fluid-permeable expansion conduits therethrough; and
depositing the foreshortened web between the two mutually opposite surfaces such that each of the surfaces contacts one side of the web, thereby retaining the crepe in those portions of the foreshortened web which do not correspond to the expansion conduits.

3. The process according to Claims 1 and 2, further comprising steps of
providing a working surface structured and configured to receive the foreshortened web thereon and having fluid-permeable expansion conduits therethrough;
providing a pressing surface opposite to the working surface, the working surface and the pressing surface being structured and configured to impress the foreshortened web therebetween;
providing a supporting surface such that the working surface is disposed between the supporting surface and the pressing surface;
disposing the foreshortened web on the working surface;
adding moisture to at least selected portions of the foreshortened web, which selected portions correspond to the expansion conduits of the working surface;
constraining the web between the working surface and the pressing surface In the direction substantially perpendicular to the working surface, thereby retaining the crepe in those portions of the foreshortened web, which portions do not correspond to the expansion conduits; and
creating a temperature differential between the working surface and the supporting surface, preferably the temperature of the pressing surface being greater than the temperature of the supporting surface, wherein the temperature differential is sufficient to cause the moisture added to the selected portions of the foreshortened web to move therethrough, thereby relaxing the crepe in the web's selected portions corresponding to the deflection conduits.

4. The process according to Claims 1, 2, and 3, further comprising a step of deflecting, under pressure, the moistened selected portions of the foreshortened web, thereby facilitating expansion of the selected portions of the web.

5. The process according to Claims 1, 2, 3, and 4, wherein the step of retaining the crepe comprises adhering the surface-contacting portions of the foreshortened web to the working surface thereby preventing lateral movement of the surface-contacting portions of the web.

6. The process according to Claims 1, 2, 3, 4, and 5, wherein the step of adding moisture to at least selected portions of the web comprises steps of:
providing steam, and
directing the steam through at least the selected portions of the web, thereby facilitating relaxation of the crepe therein.

7. The process according to Claims 1, 2, 3, 4, 5, and 6, further comprising a step of re-foreshortening the web.

8. The process according to Claims 1, 2, 3, 4, 5, 6, and 7, wherein in the step of adding moisture to at least selected portions of the web the moisture comprises substances selected from the group consisting of functional papermaking additives.

9. An apparatus for increasing bulk of a foreshortened web, the apparatus comprising:
a working surface (20) designed to receive thereon a foreshortened web comprising crepe;
a means for adding moisture to at least selected portions of the foreshortened web; and
a means for retaining the crepe in the rest of the web.

10. The apparatus according to Claim 9, wherein the working surface has a plurality of fluid-permeable expansion conduits therethrough.

11. The apparatus according to Claims 9 and 10, further comprising a pressing surface opposite to the working surface and designed to contact the foreshortened web disposed on the working surface.

12. The apparatus according to Claims 9, 10, and 11, wherein the pressing surface comprises projected areas, preferably the projected areas of the pressing surface being registered with the expansion conduits of the working surface.

13. The apparatus according to Claims 9, 10, 11, and 12, wherein the pressing surface has expansion conduits therethrough, preferably the expansion conduits of the pressing surface being registered with the expansion conduits of the working surface.

14. The apparatus according to Claims 9, 10, 11, 12, and 13, further comprising
a supporting surface associated with the working surface such that the working surface is disposed between the supparting surface and the pressing surface while facing the pressing surface; and
a means for creating a temperature differential between the pressing surface and the supporting surface, the temperature differential being sufficient to cause the moisture added to the selected portions of the web to travel therethrough, thereby relaxing the crepe in the selected portions of the web.

15. The apparatus according to Claims 9, 10, 11, 12, 13, and 14, wherein the temperature differential Is from about 50°F to about 212°F, preferably the temperature of the pressing surface being greater than the temperature of the supporting surface, the temperature differential causing the moisture added to at least the selected portions of the web to move in the direction from the pressing surface toward the supporting surface.

16. The apparatus according to Claims 9, 10, 11, 12, 13, 14, and 15, wherein the means for adding moisture to at least the selected portions of the foreshortened web comprises a sintered layer, the sintered layer preferably comprising the pressing surface.

17. The apparatus according to Claims 9, 10, 11, 12, 13, 14, 15, and 16, wherein the means for adding moisture to at least the selected portions of the foreshortened web comprises steam.

18. The apparatus according to Claims 9, 10, 11, 12, 13, 14, 15, 16, and 17, wherein each of the pressing surface, the working surface, and the supporting surface comprises an endless belt or band structured and configured to continuously travel in a machine direction.

## Patentansprüche

1. Verfahren zur Erhöhung der Fülligkeit einer verkürzten Bahn, wobei das Verfahren die folgenden Schritte umfasst:
(a) Bereitstellen einer verkürzten Bahn, die Krepp aufweist und eine allgemeine Ebene hat;
(b) Hinzufügen von Feuchtigkeit zu mindestens ausgewählten Teilen der
verkürzten Bahn, um somit eine Entspannung des Krepp in den ausgewählten Teilen der Bahn und eine Expansion der ausgewählten Teile der Bahn aus der allgemeinen Ebene der Bahn zu verursachen; und
(c) Halten des Krepp im Rest der Bahn.

2. Verfahren nach Anspruch 1, wobei es weiter folgende Schritte umfasst:
Bereitstellen zweier einander gegenüber liegenden Oberflächen, die gestaltet sind, um die verkürzte Bahn zwischen sich aufzunehmen, wobei mindestens eine der Oberflächen eine Vielzahl von fluiddurchlässigen Dehnungskanälen durch sie hindurch aufweist; und
Ablagern der verkürzten Bahn zwischen den beiden einander gegenüber liegenden Oberflächen, so dass jede der Oberflächen eine Seite der Bahn berührt, um somit den Krepp in solchen Teilen der verkürzten Bahn, die nicht den Dehnungskanälen entsprechen, aufrecht zu halten.

3. Verfahren nach den Ansprüchen 1 und 2, wobei es weiter folgende Schritte umfasst:
Bereitstellen einer Arbeitsoberfläche, die strukturiert und konfiguriert ist, um die verkürzte Bahn auf sich aufzunehmen, und die durch sie hindurch laufende fluiddurchlässige Dehnungskanäle aufweist;
Bereitstellen einer Pressoberfläche gegenüber der Arbeitsoberfläche, wobei die Arbeitsoberfläche und die Pressoberfläche strukturiert und konfiguriert sind, um die verkürzte Bahn zwischen sich zu pressen;
Bereitstellen einer Stützoberfläche, so dass die Arbeitsoberfläche zwischen der Stützoberfläche und der Pressoberfläche angeordnet ist;
Anordnen der verkürzten Bahn auf der Arbeitsoberfläche;
Hinzufügen von Feuchtigkeit zu mindestens ausgewählten Teilen der verkürzten Bahn, wobei die ausgewählten Teilen den Dehnungskanälen der Arbeitsoberfläche entsprechen;
Einzwängen der Bahn zwischen der Arbeitsoberfläche und der Pressoberfläche in einer Richtung, die im wesentlichen rechtwinklig zur Arbeitsoberfläche verläuft, um somit den Krepp in solchen Teilen der verkürzten Bahn, die nicht den Dehnungskanälen entsprechen, aufrecht zu halten; und
Schaffen einer Temperaturdifferenz zwischen der Arbeitsoberfläche und der Stützoberfläche, wobei vorzugsweise die Temperatur der Pressoberfläche größer als die Temperatur der Stützoberfläche ist, wobei die Temperaturdifferenz ausreichend ist, um zu bewirken, dass die Feuchtigkeit, die den ausgewählten Teilen der verkürzten Bahn hinzugefügt wurde, durch sie hindurch geht, um somit den Krepp in den ausgewählten Teilen der Bahn, die den Ablenkkanälen entsprechen, zu entspannen.

4. Verfahren nach den Ansprüchen 1, 2 und 3, wobei es weiter einen Schritt der unter Druck erfolgten Ablenkung der befeuchteten ausgewählten Teile der verkürzten Bahn umfasst, um somit die Ausdehnung der ausgewählten Teile der Bahn zu erleichtern.

5. Verfahren nach den Ansprüchen 1, 2, 3 und 4, wobei der Schritt des Haltens des Krepp ein Anhaften der die Oberfläche berührenden Teile der verkürzten Bahn an der Arbeitsoberfläche umfasst, um somit seitliche Bewegung der die Oberfläche berührenden Teile der Bahn zu verhindern.

6. Verfahren nach den Ansprüchen 1, 2, 3, 4 und 5, wobei der Schritt des Hinzufiigens von Feuchtigkeit zu mindestens ausgewählten Teilen der Bahn folgende Schritte umfasst:
das Liefern von Dampf; und
das Richten des Dampfs durch mindestens die ausgewählten Teile der Bahn, um somit die Entspannung des Krepp in diesen zu erleichtern.

7. Verfahren nach den Ansprüchen 1, 2, 3, 4, 5 und 6, wobei es weiter einen Schritt einer erneuten Verkürzung der Bahn umfasst.

8. Verfahren nach den Ansprüchen 1, 2, 3, 4, 5, 6 und 7, wobei im Schritt des Hinzufügens von Feuchtigkeit zu mindestens ausgewählten Teilen der Bahn die Feuchtigkeit Substanzen umfasst, die aus der Gruppe ausgewählt wurden, die aus funktionellen Zusatzstoffen der Papierherstellung besteht.

9. Vorrichtung für das Erhöhen der Fülligkeit einer verkürzten Bahn, wobei die Vorrichtung folgendes umfasst:
eine Arbeitsoberfläche (20), die gestaltet ist, um auf sich eine verkürzte Bahn, die Krepp aufweist, aufzunehmen;
eine Vorrichtung für das Hinzufügen von Feuchtigkeit zu mindestens ausgewählten Teilen der verkürzten Bahn; und
eine Vorrichtung für das Halten des Krepp im Rest der Bahn.

10. Vorrichtung nach Anspruch 9, wobei die Arbeitsoberfläche eine Vielzahl von fluiddurchlässigen Dehnungskanälen, die durch sie hindurch gehen, aufweist.

11. Vorrichtung nach den Ansprüchen 9 und 10, wobei sie weiter eine Pressoberfläche gegenüber der Arbeitsoberfläche aufweist, wobei sie gestaltet ist, um die verkürzte Bahn, die auf der Arbeitsoberfläche angeordnet ist, zu berühren.

12. Vorrichtung nach den Ansprüchen 9, 10 und 11, wobei die Pressoberfläche vorstehende Gebiete umfasst, wobei die vorstehenden Gebiete der Pressoberfläche vorzugsweise mit den Dehnungskanälen der Arbeitsoberfläche ausgerichtet sind.

13. Vorrichtung nach den Ansprüchen 9, 10, 11 und 12, wobei die Pressoberfläche Dehnungskanäle, die durch sie hindurch laufen, aufweist, wobei vorzugsweise die Dehnungskanäle der Pressoberfläche mit den Dehnungskanälen der Arbeitsoberfläche ausgerichtet sind.

14. Vorrichtung nach den Ansprüchen 9, 10, 11, 12 und 13, wobei sie weiter folgendes umfasst:
eine Stützoberfläche, die mit der Arbeitsoberfläche verbunden ist, so dass die Arbeitsoberfläche zwischen der Stützoberfläche und der Pressoberfläche angeordnet ist, während sie zur Pressoberfläche weist; und
eine Vorrichtung für das Schaffen einer Temperaturdifferenz zwischen der Pressoberfläche und der Stützoberfläche, wobei die Temperaturdifferenz ausreicht, um zu bewirken, dass die Feuchtigkeit, die ausgewählten Teilen der Bahn hinzugefügt wurde, durch sie hindurch wandert, um somit den Krepp in den ausgewählten Teilen der Bahn zu entspannen.

15. Vorrichtung nach den Ansprüchen 9, 10, 11, 12, 13 und 14, wobei die Temperaturdifferenz im Bereich von ungefähr 50°F bis ungefähr 212°F liegt, wobei vorzugsweise die Temperatur der Pressoberfläche größer als die Temperatur der Stützoberfläche ist, wobei die Temperaturdifferenz bewirkt, dass die Feuchtigkeit, die zumindest den ausgewählten Teilen der Bahn hinzugefügt wurde, sich in Richtung von der Pressoberfläche zur Stützoberfläche bewegt.

16. Vorrichtung nach den Ansprüchen 9, 10, 11, 12, 13, 14 und 15, wobei die Vorrichtung für das Hinzufügen von Feuchtigkeit zu zumindest den ausgewählten Teilen der verkürzten Bahn eine gesinterte Schicht umfasst, wobei die gesinterte Schicht vorzugsweise die Pressoberfläche umfasst.

17. Vorrichtung nach den Ansprüchen 9, 10, 11, 12, 13, 14, 15 und 16, wobei die Vorrichtung für das Hinzufügen von Feuchtigkeit zu zumindest den ausgewählten Teilen der verkürzten Bahn Dampf umfasst.

18. Vorrichtung nach den Ansprüchen 9, 10, 11, 12, 13, 14, 15, 16 und 17, wobei die Pressoberfläche, die Arbeitsoberfläche und die Stützoberfläche jeweils einen endlosen Riemen oder ein Band umfassen, die so strukturiert und konfiguriert sind, dass sie sich kontinuierlich in Maschinenrichtung bewegen.

## Revendications

1. Procédé pour augmenter le volume d'une nappe raccourcie, le procédé comprenant les étapes de :
(a) fournir une nappe raccourcie comprenant du crêpe et ayant un plan général ;
(b) ajouter de l'humidité à au moins des parties sélectionnées de la nappe raccourcie, provoquant ainsi la relaxation du crêpe dans les parties sélectionnées de la nappe et l'expansion des parties sélectionnées de la nappe vers l'extérieur à partir du plan général de la nappe ; et
(c) maintenir le crêpe dans le reste de la nappe.

2. Procédé selon la revendication 1, comprenant en outre les étapes de :
fournir deux surfaces mutuellement opposées conçues pour recevoir la nappe raccourcie entre celles-ci, au moins une des surfaces possédant une pluralité de conduits d'expansion perméables aux fluides à travers celle-ci ; et
déposer la nappe raccourcie entre les deux surfaces mutuellement opposées de telle sorte que chacune des surfaces entre en contact avec un côté de la nappe, retenant ainsi le crêpe dans ces parties de la nappe raccourcie qui ne correspondent pas aux conduits d'expansion.

3. Procédé selon les revendications 1 et 2, comprenant en outre les étapes de
fournir une surface de travail structurée et configurée pour recevoir la nappe raccourcie sur celle-ci et possédant des conduits d'expansion perméables aux fluides à travers celle ci ;
fournir une surface de pression opposée à la surface de travail, la surface de travail et la surface de pression étant structurées et configurées pour imprimer la nappe raccourcie entre celles-ci ;
fournir une surface d'appui de telle façon que la surface de travail soit disposée entre la surface d'appui et la surface de pression ;
disposer la nappe raccourcie sur la surface de travail ;
ajouter de l'humidité à au moins des parties sélectionnées de la nappe raccourcie, lesquelles parties sélectionnées correspondent aux conduits d'expansion de la surface de travail ;
retenir la nappe entre la surface de travail et la surface de pression dans la direction sensiblement perpendiculaire à la surface de travail, retenant ainsi le crêpe dans ces parties de la nappe raccourcie, lesquelles parties ne correspondent pas aux conduits d'expansion ; et
créer un différentiel de température entre la surface de travail et la surface d'appui, la température de la surface de pression étant de préférence supérieure à la température de la surface d'appui, dans lequel le différentiel de température est suffisant pour permettre à l'humidité ajoutée aux parties sélectionnées de la nappe raccourcie de pénétrer à travers celles-ci, entraînant ainsi la relaxation du crêpe dans les parties sélectionnées de la nappe correspondant aux conduits de déflexion.

4. Procédé selon les revendications 1, 2 et 3, comprenant en outre une étape de déflexion, sous pression, des parties sélectionnées humidifiées de la nappe raccourcie, facilitant ainsi l'expansion des parties sélectionnées de la nappe.

5. Procédé selon les revendications 1, 2, 3 et 4, dans lequel l'étape de rétention du crêpe comprend l'adhérence à la surface de travail des parties de la nappe raccourcie en contact avec la surface, empêchant ainsi le mouvement latéral des parties de la nappe en contact avec la surface.

6. Procédé selon les revendications 1, 2, 3, 4 et 5, dans lequel l'étape d'ajout d'humidité à au moins des parties sélectionnées de la nappe comprend les étapes de :
fournir de la vapeur et
diriger la vapeur à travers au moins les parties sélectionnées de la nappe, facilitant ainsi la relaxation du crêpe dans celles-ci.

7. Procédé selon les revendications 1, 2, 3, 4, 5, et 6, comprenant en outre une étape de raccourcir à nouveau la nappe.

8. Procédé selon les revendications 1, 2, 3, 4, 5, 6 et 7, dans lequel dans l'étape d'ajout d'humidité à au moins des parties sélectionnées de la nappe, l'humidité comprend des substances sélectionnées parmi le groupe constitué par les additifs fonctionnels de fabrication du papier.

9. Appareil pour augmenter le volume d'une nappe raccourcie, l'appareil comprenant :
une surface de travail (20) conçue pour recevoir sur celle-ci une nappe raccourcie comprenant du crêpe ;
un moyen pour ajouter de l'humidité à au moins des parties sélectionnées de la nappe raccourcie ; et
un moyen pour retenir le crêpe dans le reste de la nappe.

10. Appareil selon la revendication 9, dans lequel la surface de travail possède une pluralité de conduits d'expansion perméables aux fluides à travers celle-ci.

11. Appareil selon les revendications 9 et 10, comprenant en outre une surface de pression opposée à la surface de travail et conçue pour être en contact avec la nappe raccourcie disposée sur la surface de travail.

12. Appareil selon les revendications 9, 10 et 11, dans lequel la surface de pression comprend des zones projetées, les zones projetées de la surface de pression coïncidant de préférence avec les conduits d'expansion de la surface de travail.

13. Appareil selon les revendications 9, 10, 11 et 12, dans lequel la surface de pression possède des conduits d'expansion à travers celle-ci, les conduits d'expansion de la surface de pression coïncidant de préférence avec les conduits d'expansion de la surface de travail.

14. Appareil selon les revendications 9, 10, 11, 12 et 13, comprenant en outre
une surface d'appui associée à la surface de travail de telle sorte que la surface de travail soit disposée entre la surface d'appui et la surface de pression tout en faisant face à la surface de pression ; et
un moyen pour créer un différentiel de température entre la surface de pression et la surface d'appui, le différentiel de température étant suffisant pour permettre à l'humidité ajoutée aux parties sélectionnées de la nappe de passer à travers celles-ci, entraînant ainsi la relaxation du crêpe dans les parties sélectionnées de la nappe.

15. Appareil selon les revendications 9, 10, 11, 12, 13 et 14, dans lequel le différentiel de température est d'environ 50°F à environ 212°F, la température de la surface de pression étant de préférence supérieure à la température de la surface d'appui, le différentiel de température permettant à l'humidité ajoutée au moins aux parties sélectionnées de la nappe de se déplacer depuis la surface de pression vers la surface d'appui.

16. Appareil selon les revendications 9, 10, 11, 12, 13, 14 et 15, dans lequel le moyen pour ajouter de l'humidité au moins aux parties sélectionnées de la nappe raccourcie comprend une couche frittée, la couche frittée comprenant de préférence la surface de pression.

17. Appareil selon les revendications 9, 10, 11, 12, 13, 14, 15 et 16, dans lequel le moyen pour ajouter de l'humidité au moins aux parties sélectionnées de la nappe raccourcie comprennent de la vapeur.

18. Appareil selon les revendications 9, 10, 11, 12, 13, 14, 15, 16 et 17, dans lequel chacune de la surface de pression, de la surface de travail et de la surface d'appui comprend une courroie ou bande sans fin structurée et configurée pour se déplacer en continu dans une direction de la machine.
